

## UNITED STATES PATENT OFFICE

2,098,063

## PROCESS FOR DEOXIDATION OF COPPER

René Perrin, Paris, France, assignor to Société d'Electrochimie d'Electrometallurgie et des Acierées Electriques d'Ugine, Paris, France, a corporation of France

No Drawing. Application June 7, 1937, Serial No. 146,964. In France June 16, 1936

4 Claims. (Cl. 75—76)

It is already known to deoxidize copper by causing to act upon this metal in the molten state various reactive substances which act to extract from the copper the oxygen which it contains, in particular in the form of copper oxide.

5 The operation is effected either by placing the molten metal in a heated furnace and by placing above a deoxidizing flux or slag which is caused to act for the time necessary, or by introducing 10 the flux into the pouring jet of the copper or into the ladle into which the copper is poured, or by causing the copper to flow through the molten flux placed in a crucible, or again by violently intermixing the liquid copper with a 15 flux or slag capable of absorbing the copper oxides, this intermixing being for example effected by violently pouring the copper for example in a large jet upon a slag molten in advance in the bottom of a ladle, the size of the jet and the 20 height from which the metal is poured being such that the slag forms a sort of emulsion in the metal and that the operation of deoxidation is almost instantaneous, according to the process previously patented by applicant for purifying 25 copper by violent intermixing of molten fluid slag and metal.

The present invention has for subject the application of metaphosphoric acid to the deoxidation of copper by an operation of the kind of those 30 mentioned above. Metaphosphoric acid has been found in fact to be a particularly active flux which permits in a short time considerable quantities of oxygen to be extracted from molten copper.

The employment of this substance may take

place by any of the means indicated above for the use of the usual fluxes. Metaphosphoric acid may be put either in the solid state or in the liquid state into contact with the copper.

*Example*

5

In a crucible, 20 kgs. of copper was melted. The bath when formed had an oxygen content of 0.20%. To the bath, 1 kg. of metaphosphoric acid was added and allowed to melt and to act on 10 the metal for about 15 minutes. After this period of action the oxygen content of the metal had fallen to 0.020%.

I claim:

1. Process for deoxidation of copper by the 15 action of a deoxidizing flux consisting in causing metaphosphoric acid to act upon a bath of oxidized copper.

2. Process for deoxidation of copper by the action of a deoxidizing flux consisting in causing 20 metaphosphoric acid to act upon the molten copper by putting it into contact in the solid state with the copper.

3. Process for deoxidation of copper by the action of a deoxidizing flux consisting in causing 25 metaphosphoric acid to act upon the molten copper by putting it into contact in the liquid state with the copper.

4. Process for deoxidation of copper by the action of a deoxidizing flux consisting in causing 30 metaphosphoric acid to act upon the molten copper by violently intermixing the metaphosphoric acid and the copper.

RENE PERRIN.